

## UNITED STATES PATENT OFFICE.

ROBERT HOWSON PICKARD, DOROTHY JORDAN LLOYD, AND ALBERT EDWARD CAUNCE,  
OF LONDON, ENGLAND.

## MANUFACTURE OF LEATHER.

No Drawing. Application filed August 22, 1925, Serial No. 51,874, and in Great Britain August 27, 1924.

This invention has reference to improvements in and relating to the manufacture of leather.

This may be effected either by steeping the 5 prepared and wet skin, hide, or pelt (all hereinafter included in the term skin) in a liquid tanning material or by subjecting it to the action of formaldehyde gas which latter, being readily soluble in water, is thus 10 made to permeate the wet skin in the form of a solution.

Our invention differs essentially from the foregoing in that we effect the tanning by a 15 tanning agent in gaseous form which remains in that form throughout the tanning operation.

An important feature of our invention is 20 that we first dehydrate the skin and then subject the dehydrated or dried skin to the action of a tanning agent in gaseous form.

The dehydration should be effected without 25 bringing about shrinkage of the fibres of the skin and to this end we immerse the wet skin in a bath or may be successive baths of a volatile solvent of water not injurious to the fibres of the skin and then evaporate off the solvent. Acetone is a solvent of water eminently suitable 30 for the purpose.

Instead of immersing the skin in a bath we 35 may spray it with the solvent to effect its dehydration.

Formaldehyde vapour, or an inert gas or air saturated with formaldehyde, constitutes 40 an excellent tanning agent when employed for effecting the tanning of dehydrated skins, but we wish it to be understood that our invention is not limited to this as other aldehydes (such 45 as acetaldehyde), bromine, chlorine, or any of the numerous substances which are known to tan in aqueous or alcoholic solution but which can also be conveniently and economically converted into their gaseous forms, may be employed in carrying our invention into practice.

When the dehydration of the skin has been 50 effected, for instance by steeping it in successive baths of acetone of suitable strength and then evaporating off the acetone in the skin, the dry skin which is very porous is subjected 55 to the action of a tanning agent in gaseous form and, owing to the porosity of the dry skin, said agent will readily permeate it and if the treatment be continued thorough tan-

The skin thus converted into leather may now be dyed, stuffed, fat liquored, or subjected to any other usual and desired finishing operation.

We now propose—by way of examples—to 60 describe in greater detail the method to be adopted when goat pelt and skin in the hair are to be tanned in accordance with our invention, the details appertaining to the treatment of these being sufficient to enable those 65 skilled in the art to make the necessary variations if different primary materials than those stated (for instance hide) are to be tanned.

In the case of goat pelt, this in the bated 70 condition is washed with cold water and is then dried by treatment with or in a bath or a succession of baths of acetone until in the final bath the pelt is in equilibrium with a mixture of water and acetone of density not 75 greater than 0.810. (The thoroughness of the treatment can be conveniently tested by cutting off a small piece of the pelt and if this after evaporation off of the acetone at 135° Fah. (57° cent.) wets back rapidly with 80 water the treatment is complete). The excess of acetone is then drained off and the acetone remaining in the pelt evaporated in a current of air or inert gas which may be heated up to a convenient temperature of 85 135° Fah. (57° cent.).

The pelt so prepared may at once be subjected to the further treatment to be described, or it may be stored until it is convenient to treat it.

The further treatment consists in packing or suspending the pelt in the above very porous condition in a suitable container through which, by suction or pressure, is passed a current of air or inert gas containing mixed with 95 it the formaldehyde or other tanning agent in the gaseous or vapour state. A suitable mixture is obtained by bubbling the air through a solution of formalin in water which may be warmed. Or the formaldehyde may be used 100 in the gaseous form without admixture with air.

The treatment of the pelt with the tanning agent in gaseous form will be continued for some time (depending upon the thickness and character of the pelt) and owing to the very porous condition of the pelt the said tanning agent in gaseous form will readily penetrate and permeate it and comparatively rapidly 105 completely change it into leather.

The leather thus produced retains its substance, that is to say it loses nothing or at any rate very little in volume as compared with the pelt in wet condition. It may now be removed for any usual further finishing process such as fatliquoring and owing to its great porosity the absorption of the fatliquor takes place very readily and a very white and supple leather will result.

10 It is of course essential that the treatment with the tanning agent in gaseous form be continued long enough to complete the tannage and this may conveniently be determined by testing a sample piece by "wetting back" with water and then drying out. If the "wet back" test piece retains its substance and white opaque appearance after it is dried out in air, the tannage is complete.

20 When haired skins are to be tanned in accordance with our invention we proceed as follows:

25 The skins, after preliminary wet work such as washing "soaking back" with water or the like, and the usual short amount of treatment with alkalies such as caustic soda in dilute solution of lime, is then "de-limed" with weak dilute acid solution such as borasic acid, so that the skin is in equilibrium with a solution of reaction pH about that usually used in the bathing operation, namely between pH=5.5 and pH=8.5 preferably pH=7. The skins may then be washed with water if desired, and then dried by the process of acetone treatment previously described.

35 The skin so prepared is then subjected to the action of the tanning agent in gaseous form as in the case of goat pelt and the sufficiency of the treatment may be ascertained by a similar test.

40 The tanning completed the resultant leather is eminently suited for dyeing, fatliquoring, and/or other usual finishing treatment.

45 By subjecting skin in the hair to the complete treatment described to effect its tannage, the risk of the hair becoming loose is materially reduced as it is not necessary to maintain the skin in wet condition for such a long time as is necessary for example when 50 wool rugs or furs are prepared by known methods. Further, the drying by acetone and treatment with formaldehyde in the gaseous state will tend to keep the skin sterile and to disinfect it, and withal the product, viz, 55 wool rug or fur, will be softer and therefore more supple than those whereof the haired skin is treated in the known manner.

We claim:

1. The manufacture of leather by subjecting a dehydrated skin to the action of formaldehyde vapor.

2. The manufacture of leather by removing from a skin its water content by immersing the wet skin in acetone and then evaporating off the acetone so as to leave the fibres of the skin in the open condition, and then subjecting it to the action of formaldehyde vapour.

3. The manufacture of leather by treating 70 a skin with acetone, evaporating off the acetone from the skin, and then subjecting the skin to the action of formaldehyde vapor.

4. The manufacture of leather by immersing a skin in acetone until it is in equilibrium 75 with a mixture of acetone and water of specific gravity not greater than 0.810, evaporating off the acetone from the skin and subjecting it to the action of formaldehyde vapor.

80 5. A process of manufacturing leather according to which the tannage of the leather is effected by treatment whilst in dry condition with formaldehyde vapour which is in gaseous form throughout the tanning operation.

ROBERT HOWSON PICKARD.

DOROTHY JORDAN LLOYD.

ALBERT EDWARD CAUNCE.